

## UNITED STATES PATENT OFFICE.

PAUL BALKE AND GUSTAV LEYSIEFFER, OF TROISDORF, GERMANY.

## PHONOGRAPHIC RECORD.

No Drawing. Application filed December 1, 1920, Serial No. 427,635, and in Germany February 13, 1920.

- The phonographic records for talking machines and the like which are now in vogue are at the present produced entirely of a substance whose principal component is shellac. 5 These records possess a number of serious drawbacks, as for example the impure tone which arises through the injuries done to the phonetic impressions when the records are used a number of times, the high price 10 of the records or plates, due to the shellac that has to be imported. Further drawbacks are the great weight of the plates, their exceedingly great frangibility and the imperfect reproduction of the music as regards the 15 clearness and fulness of the sound. It is true that attempts have already been made to use other materials for producing sound records, but no record of practical value has as yet been produced without shellac. 20 Another idea in this connection is disclosed in the German Patent No. 267,161. In accordance with this, shellac cannot be dispensed with, but it is considered to be a progressive step to enable the use of shellac 25 or the like to be restricted to the core, whilst the outside coating of the same is made of cellulose esters or mixtures thereof. But these composite plates do not fulfil the requirements met by a homogenous sound 30 record and have not appeared upon the market. Besides, even these plates require a large amount of shellac which, if it can be got at all, under the conditions prevailing at the present day, is so difficult to procure that the avoidance of this raw material 35 is a matter of great economic importance. 40 The present invention consists in providing a non-composite, homogeneous, uniform, sound record made of cellulose esters and a considerable admixture of finely ground filling substance and an admixture of gelatinizing agents. The proportionate quantities of the said three components of the substance of which the plate is formed is such that the 45 amount of gelatinizing agent in the mixture is larger than the quantity needed for the actual gelatinizing of the cellulose or its derivatives. Records made of such substances attain the qualities of the known best shellac plates in every respect, and surpass 50 them in regard to the fullness and purity of the emitted tone. They are very elastic, in-frangible, of a very light weight and, as has already been pointed out, cost little to produce, because the materials that are hard to 55 procure are dispensed with.
- Experiments have shown that fibrous substances (cellulose, cotton, peat, cork and the like) make particularly good filling agents. A process for producing records or plates 60 of this kind will now be described by way of example:
- The finely-ground filling substance is added to the cellulose esters or other derivatives, the quantity of the said substance exceeding that of the basic material employed. Suitable gelatinizing agents are added to this mixture, the quantity of these agents being larger than that which is needed for 65 gelatinizing the cellulose ester. The whole 70 is then worked up into a homogeneous mass which is rolled out into sheets. Plates are then stamped out of the sheets and finally the sound records are impressed on the plates. A specific example of a mixture 75 showing the actual amounts of the components used is the following:
- |                            |    |
|----------------------------|----|
| 35 kgs. nitro-cellulose.   | 80 |
| 42 kgs. cellulose.         |    |
| 5 kgs. black earth-colour. |    |
- |                                                                                                                                                                                                                                                                                                                                                                   |    |
|-------------------------------------------------------------------------------------------------------------------------------------------------------------------------------------------------------------------------------------------------------------------------------------------------------------------------------------------------------------------|----|
| 18 kgs. gelatinizing agent, such as methyl, ethyl, urea.                                                                                                                                                                                                                                                                                                          | 85 |
| Our invention broadly comprises the provision of a homogeneous sound record having as its essential ingredients a cellulose ester or an ester of a cellulose derivative, a gelatinizing agent, and a filling agent. In the above example, nitro-cellulose is given as an example of the cellulose constituent and methyl ethyl urea of the gelatinizing 90 agent. |    |
- We claim:
1. A homogeneous sound record for talking machines or the like consisting of cellulose nitrate, a filling material, and a gelatinizing agent, the filling material being present in a quantity greater than the cellulose nitrate, and the gelatinizing agent in a quantity greater than that required to gelatinize the nitrate.
  2. A homogeneous sound record for talking machines or the like consisting of cellul-

lose nitrate, a filling material and methyl ethyl urea adapted to act as a gelatinizing agent.

3. A homogeneous sound record for talking machines or the like consisting of a cellulose nitrate, a filling material and methyl ethyl urea adapted to act as a gelatinizing agent, the filling material being present in

a quantity greater than the cellulose nitrate and the methyl ethyl urea in a quantity 10 greater than that required to gelatinize the nitrate.

In testimony whereof we affix our signatures.

DR. PAUL BALKE.

DR. GUSTAV LEYSIEFFER.